

## UNITED STATES PATENT OFFICE

2,450,321

## RUST-INHIBITING GREASES

Ernest T. White, Jackson Heights, and Reuben Carl Robinson, New York, N. Y., assignors to Socony-Vacuum Oil Company, Incorporated, a corporation of New York

No Drawing. Application April 9, 1947,  
Serial No. 740,495

14 Claims. (Cl. 252—42)

1

This invention relates to improved lubricating compositions and, more particularly, to rust-inhibiting grease compositions.

It is well known that moisture, even in the presence of lubricants, has a tendency to corrode steel, iron, and other metal parts with which it comes in contact. Corrosion of this type is particularly prevalent and troublesome in the operation of steam turbines where steam or water is in continual contact with almost all parts of the turbine system. As is readily apparent, corrosion and rusting of the metallic parts of such systems and other similar precision-built machinery is to be strictly avoided. It is highly desirable, therefore, to prepare lubricants which offer substantial resistance to rust formation in the presence of water. In the case of marine turbines, the lubricant employed should also prevent rusting in the presence of sea water.

Greases employed for the lubrication of steam turbines and other machinery which is much in contact with water have heretofore been treated with certain rust-preventive agents, such as metallic sulfonates and the like, which have the property of permitting the metallic surface to be preferentially coated with lubricant instead of water, thus preventing or substantially reducing the actual contact of the water with the metal surface and the ensuing rust formation. An objectionable feature resulting from the use of metallic sulfonates and similar water-soluble compositions has been the tendency of such materials to render a grease, containing the same, water-absorbent. This undesirable phenomena, in turn, causes a change in structure of the grease and leads to the formation of an emulsion of the grease and water, thereby thinning out the grease and substantially reducing its lubricating efficiency.

It is an object of the present invention to provide grease compositions which are free from the above described emulsion-forming tendency and which, at the same time, offer substantial resistance to rust formation in the presence of water.

The aforesaid object is accomplished in accordance with the present invention by the provision of a grease containing a small amount of a compound characterized by the general formula:



where R is an aromatic nucleus of the benzene, anthracene, phenanthrene, naphthalene or other condensed ring series, and Y is an aliphatic, cycloaliphatic, arylaliphatic or aryl group having at least four carbon atoms. Representative of the

2

compounds contemplated for use as rust-preventive additives in greases of this invention are substituted phenoxy tetraethoxy ethanols, substituted naphthoxy tetraethoxy ethanols, substituted anthroxy tetraethoxy ethanols, substituted phenanthroxy tetraethoxy ethanols, and the like, wherein at least one of the substituents in the aromatic nucleus is a group such as butyl, amyl, hexyl, octyl, dodecyl, tetradecyl, hexadecyl, oleyl or other alkyl group containing up to 30 carbon atoms; a cycloaliphatic group, such as cyclohexyl, octyl-cyclohexyl, lauryl-cyclohexyl, cetyl-cyclohexyl, butyl-cyclohexyl, etc.; bornyl, abietyl, decahydronaphthyl, tetrahydro-abietyl, or other terpenic radical or a naphthenic radical; phenyl, benzyl, phenylethyl, phenylisobutyl or other aryl or arylaliphatic hydrocarbon group. The substituents above mentioned may have straight or branched chains and the aromatic nucleus of the 10 above defined compounds may have more than one substituent which may either be the same or a different group. In general, when more than one substituent is present in the aromatic nucleus of the above compounds, at least one of the substituents will contain four or more carbon atoms; the remaining substituent or substituents may then optionally contain less than four carbon atoms and be represented by methyl, ethyl, propyl, isopropyl radicals, and the like.

It has been found, as a general rule, that the di- and poly-substituted compounds of the type described above are more effective in inhibiting rust formation when incorporated in greases than the mono-substituted compounds. The use of the 20 former type compounds accordingly represents a preferred embodiment of this invention. In particular, the substituted phenoxy tetraethoxy ethanols are suitably employed as rust-preventive additives in the greases of the present invention.

Of the various substituent groups, preference is accorded those compounds containing alkyl substituents.

The above described compounds may be suitably prepared by condensing a phenolic compound 25 corresponding to the formula:



with a compound of the type:



in which X is a halogen atom, said condensation taking place in the presence of an alkali to split out an alkali metal halide and thus yield the desired inhibitor.

55 The greases containing one or more of the

aforesaid compounds are the alkali metal base greases, that is, grease compositions consisting basically of mineral oils in admixture with alkali metal soaps of fatty acids or with a sufficient proportion of such alkali metal soaps present to give to the greases the characteristics usually recognized as attributable to alkali base greases. These greases are usually prepared by heating a fat or a fatty acid, or a mixture thereof, with a mineral oil and thereafter heating the resultant mixture with caustic soda at elevated temperatures to obtain a substantially anhydrous soda soap grease. Lithium soap greases are ordinarily made by charging a lithium soap to a grease kettle, adding mineral oil, and heating at an elevated temperature in the range of about 380 to 440° F. with agitation to prepare a homogeneous composite which is then withdrawn from the kettle and allowed to cool. The greases so prepared will generally have an alkali metal soap content of less than about 30 per cent of the final composition, and preferably between about 5 and about 20 per cent.

The mineral oil constituent of the greases contemplated herein may vary considerably in character and includes residual or distilled oils. Preference is accorded, however, to oils having a viscosity (S. U. V.) of 50-200 seconds at 100° F. The fats and fatty acids which may be employed are those generally found in alkali metal base greases. Examples of such saponifiable materials include vegetable, animal and fish fatty oils; hydrogenated fatty materials thereof; high molecular weight organic acids, such as stearic acid and oleic acid; the high molecular weight acids resulting from the oxidation of petroleum fractions; rosin and related products; high molecular weight naphthenic acids, sulfonic acids, etc.; and saponifiable waxes, such as beeswax, sperm oil, degras, and the like.

While the present invention contemplates the improvement of alkali metal base greases generally, it has been discovered that lithium base greases are rendered particularly effective as rust-inhibiting compositions by incorporation therein of small amounts of the above described inhibiting compounds. Thus, a preferred embodiment of this invention is the provision of a rust-inhibiting lithium base grease.

It has further been discovered, in accordance with this invention, that the inhibitors described hereinabove can be incorporated in the alkali metal greases during any stage of the manufacturing process before the grease is drawn from the kettle into containers to cool. The amount of inhibitor employed in the greases of the type described will normally be less than about 5 per cent of the final composition, the minimum amount to be used being about 0.1 per cent and the preferred amount between about 0.5 and about 2 per cent and, in particular, an amount of the order of 0.75 per cent.

In addition to the rust-preventive agents set forth above, various other materials may be added to the grease compositions of this invention, such as alcohols and other solvents, oxidation inhibitors, waxes, fillers, etc. Oxidation inhibitors which may be added to the grease include alkyl phosphites, phenyl alpha naphthylamine, tetra-methyl diamino diphenyl methane, benzidine, etc. Such anti-oxidants, while not essential to the production of a good grease in accordance with the present invention, are preferably employed to aid in prolonging the life of the grease and to inhibit oxidation thereof. The amount of

anti-oxidant employed may vary from about 0.001 per cent to about 1.0 per cent of the finished grease.

Various tests exist for measuring the tendency toward rust formation of lubricants. The greases of the present invention were evaluated by the salt spray method prescribed in Naval Ordnance specification O. S. 1350, section F-3b, dated June 22, 1945. Briefly, this method consists of coating a clean, polished steel panel with a uniform thin film of grease to be tested. The amount of grease so applied is such that its total weight does not exceed 0.21 gram when applied to a panel of approximately 1" x 3" x 1/8". The panels so treated are allowed to stand in a dust-free atmosphere at room temperature for 24 hours and are then exposed to a 4 per cent salt spray at about 95° F. for a specified period of time, usually not less than 100 hours. The panels are then examined for rust formation.

The following greases and results of testing in accordance with the above described procedure are illustrative of those contemplated by the present invention:

#### Example I

A slurry of 13 parts by weight of lithium stearate and 85.25 parts by weight of naphthenic oil having a viscosity (S. U. V.) of 60 seconds at 100° F. was prepared in a grease kettle. The mixture was then fire-heated with agitation at a temperature in the range of 380-410° F. When the grease was in a molten state, one part by weight of phenyl alpha naphthylamine and 0.75 part by weight of octyl methyl phenoxy tetraethoxy ethanol were added. The composition was then thoroughly stirred to mix in the anti-oxidant and inhibitor. The resultant mixture was maintained in the above temperature range for 5-10 minutes with stirring. At the end of this time, the grease was drawn into pans and allowed to cool. The solid grease was then cut into cakes of the desired size and then milled in a grease mill to a smooth, buttery, homogeneous structure. This grease is hereinafter referred to as grease I.

#### Example II

A lithium base grease was prepared as in Example I, except that, as the rust-preventive agent, 0.75 part by weight of octyl phenoxy tetraethoxy ethanol were incorporated in the grease. The grease so obtained is hereinafter referred to as grease II.

#### Example III

A grease, consisting of 15 parts by weight of a sodium salt of a hydrogenated fish oil and 84.25 parts by weight of a naphthenic oil having a viscosity (S. U. V.) of 100 seconds at 100° F., was prepared in a conventional manner in a steam-heated kettle. The fatty material was melted in a portion of the mineral oil, and the caustic soda, as a water solution, was added while agitating. The resulting mixture was dehydrated with agitation until a good soap structure was obtained, and the balance of the mineral was then added. At this point the temperature of the grease was in the range of 280-340° F., and 0.75 part by weight of octyl methyl phenoxy tetraethoxy ethanol were added. The composition was then thoroughly agitated at a temperature in the above range for a period of time sufficient to insure complete mixture of the additive with the grease. The grease was then cooled and removed from the kettle into containers. The re-

sultant grease is hereinafter referred to as grease III.

*Example IV*

A soda base grease was prepared as in Example III, except that, as the rust preventive agent, 0.75 part by weight of octyl phenoxy tetraethoxy ethanol were incorporated in the grease. The grease so obtained is hereinafter referred to as grease IV.

The above prepared greases were tested in accordance with the salt spray test described hereinabove and the following results were obtained:

|                            |                          |
|----------------------------|--------------------------|
| Uninhibited lithium grease | Heavy rust in 100 hours  |
| Grease I                   | No rusting in 100 hours  |
| Grease II                  | No rusting in 100 hours  |
| Uninhibited sodium grease  | Heavy rust in 100 hours  |
| Grease III                 | Slight rust in 100 hours |
| Grease IV                  | Slight rust in 100 hours |

A series of extended tests on lithium base greases I and II showed that panels coated with grease I could be exposed for a period of 250-300 hours to the salt spray at a temperature of 95° F. before rusting occurred. Similarly, panels coated with grease II could be exposed for a period of 150-200 hours before rusting took place. A conventional lithium base grease containing only soap, oil, and anti-oxidant, when tested under identical conditions, was found to allow rusting to occur in less than 20 hours.

These results indicate a very substantial and useful increase in rust-inhibiting properties of alkali greases, particularly lithium base greases, and considerably widen the field to which such greases may be applied, rendering them capable of use in a great number of applications in the presence of water, wherein they have formerly not been capable of use with a particularly high degree of efficiency.

It is to be further noted that the rust-inhibiting compounds of this invention are water-insoluble and while imparting rust-proofing properties to the grease, do not detract from the natural water insolubility of lithium grease itself. The maximum water absorption of a conventional lithium base grease, prepared according to the procedure set forth in Example I, but without the incorporation of octyl methyl phenoxy tetraethoxy ethanol, was found to be about 20 per cent when tested in accordance with the water-absorption test prescribed in Naval Ordnance specification O. S. 1350, section F-3h, dated June 22, 1945. With the addition of 0.75 per cent of this compound to afford over 100 hours salt spray protection, the water absorption of the grease was still only 20 per cent. When a conventional rust preventive, such as sodium sulfonate, was employed, it was found necessary to use 2 per cent of this material to secure the same salt spray protection as attained with 0.75 per cent of an inhibitor of this invention. Moreover, it was found that a grease containing sodium sulfonate absorbed over 200 per cent by weight of water and became a thin emulsion when subjected to the aforementioned water-absorption test. The grease containing the rust-inhibiting compounds of this invention showed no change in structure when brought into contact with water.

We claim:

1. An alkali metal rust-inhibiting grease comprising a major proportion of a mineral oil, an alkali metal soap present in sufficient propor-

tion to thicken said oil to a grease consistency, and between about 0.5 and about 2 per cent by weight of a compound having the general formula:



where R represents an aromatic nucleus and Y is a member selected from the group consisting of aliphatic, cycloaliphatic, arylaliphatic and aryl hydrocarbon radicals having at least four carbon atoms.

2. A lubricating grease composition characterized by resistance to rust formation, comprising a major proportion of a mineral oil, an alkali metal soap present in sufficient proportion to thicken said oil to a grease consistency, and between about 0.1 and about 5 per cent by weight of a compound having the general formula:



20 where R represents an aromatic nucleus and Y is a member selected from the group consisting of aliphatic, cycloaliphatic, arylaliphatic and aryl hydrocarbon radicals having at least four carbon atoms.

25 3. A lubricating grease composition characterized by resistance to rust formation, comprising a major proportion of a mineral oil, a lithium soap present in sufficient proportion to thicken said oil to a grease consistency, and between about 0.1 and about 5 per cent by weight of a compound having the general formula:



where R represents an aromatic nucleus and Y is 35 a member selected from the group consisting of aliphatic, cycloaliphatic, arylaliphatic and aryl hydrocarbon radicals having at least four carbon atoms.

4. A lubricating grease composition characterized by resistance to rust formation, comprising a major proportion of a mineral oil, a sodium soap present in sufficient proportion to thicken said oil to a grease consistency, and between about 0.1 and about 5 per cent by weight 45 of a compound having the general formula:



where R represents an aromatic nucleus and Y is 50 a member selected from the group consisting of aliphatic, cycloaliphatic, arylaliphatic and aryl hydrocarbon radicals having at least four carbon atoms.

5. A lubricating grease composition characterized by resistance to rust formation, comprising a major proportion of a mineral oil, a lithium soap present in sufficient proportion to thicken said oil, and between about 0.5 and 2 per cent by weight of a compound having the general formula:



60 where R represents an aromatic nucleus and Y is a member selected from the group consisting of aliphatic, cycloaliphatic, arylaliphatic and aryl hydrocarbon radicals having at least four carbon atoms.

65 6. A lubricating grease composition characterized by resistance to rust formation, comprising a major proportion of a mineral oil, an alkali metal soap present in sufficient proportion to thicken said oil to a grease consistency, and between about 0.1 and about 5 per cent by weight of an alkyl-substituted phenoxy tetraethoxy ethanol, the alkyl substituent of which contains 70 at least four carbon atoms.

7. A lubricating grease composition characterized by resistance to rust formation, comprising a major proportion of a mineral oil, a lithium soap present in sufficient proportion to thicken said oil to a grease consistency, and between about 0.1 and about 5 per cent by weight of an alkyl-substituted phenoxy tetraethoxy ethanol, the alkyl substituent of which contains at least four carbon atoms.

8. A lubricating grease composition characterized by resistance to rust formation, comprising a major proportion of a mineral oil, a lithium soap present in sufficient proportion to thicken said oil to a grease consistency and between about 0.5 and about 2 per cent by weight of an alkyl-substituted phenoxy tetraethoxy ethanol, the alkyl substituent of which contains at least four carbon atoms.

9. A lubricating grease composition characterized by resistance to rust formation, comprising a major proportion of a mineral oil, an alkali metal soap present in sufficient proportion to thicken said oil to a grease consistency, and between about 0.1 and about 5 per cent by weight of octyl methyl phenoxy tetraethoxy ethanol.

10. A lubricating grease composition characterized by resistance to rust formation, comprising a major proportion of a mineral oil, an alkali metal soap present in sufficient proportion to thicken said oil to a grease consistency, and between about 0.1 and about 5 per cent by weight of octyl phenoxy tetraethoxy ethanol.

11. A lubricating grease composition characterized by resistance to rust formation, comprising a major proportion of mineral oil, a lithium soap present in sufficient proportion to thicken said oil to a grease consistency, and between

about 0.1 and about 5 per cent by weight of octyl methyl phenoxy tetraethoxy ethanol.

12. A lubricating grease composition characterized by resistance to rust formation, comprising a major proportion of mineral oil, a lithium soap present in sufficient proportion to thicken said oil to a grease consistency, and between about 0.1 and about 5 per cent of octyl phenoxy tetraethoxy ethanol.

10 13. An alkali metal rust-inhibiting grease formed by compounding together a major proportion of a mineral oil, from 5 to 20 per cent of a high molecular weight fatty acid soap of an alkali metal and from 0.5 to 2 per cent by weight of an alkyl-substituted phenoxy tetraethoxy ethanol, the alkyl substituent containing at least four carbon atoms.

14. A lithium base rust-inhibiting grease formed by compounding together a major proportion of a mineral oil, from 5 to 20 per cent of a high molecular weight fatty acid soap of lithium and from 0.5 to 2 per cent of an alkyl-substituted phenoxy tetraethoxy ethanol, the alkyl substituent containing at least four carbon atoms.

25 ERNEST T. WHITE.  
R. CARL ROBINSON.

## REFERENCES CITED

30 The following references are of record in the file of this patent:

## UNITED STATES PATENTS

| Number       | Name                   | Date          |
|--------------|------------------------|---------------|
| 35 2,233,381 | De Groote et al. ----- | Feb. 25, 1941 |
| 2,361,043    | McCleary -----         | Oct. 24, 1944 |